

Jan. 3, 1933.

M. B. COVERT

1,893,274

METHOD OF TREATING PISTON RINGS

Filed Nov. 26, 1930

Fig. 1.



Fig. 2.



Fig. 3.



Witness:

William P. Nichols

Inventor:  
Martin B. Covert  
by M. B. Covert M.B.C.

## UNITED STATES PATENT OFFICE

MARTIN B. COVERT, OF HOLLAND, MICHIGAN, ASSIGNOR TO RENU PARTS CORPORATION, OF HOLLAND, MICHIGAN, A CORPORATION OF MICHIGAN

## METHOD OF TREATING PISTON RINGS

Application filed November 26, 1930. Serial No. 498,282.

This invention particularly relates to the manufacture of piston rings and the like.

It has been found in use of cast iron piston rings as heretofore manufactured that warping occurs, and the amount of resultant distortion of the ring depends largely upon the shape of the article and the internal strains that are set up in the process of cooling and also on the temperature of the motor in which the rings are used as well as the vibrations and jars to which the rings are subjected during operation of the motor. Such warping or distorting of the rings permits leakage past the same with the resultant detrimental effects well understood in the art. To obviate such warping it has been customary to allow the ring castings to age or set after a machining operation but this process may take from six to eight months or even longer depending almost entirely upon the size of the casting and the accuracy that is to be required of the part after the ring is completed. It has been found that unless this is done the finished rings will change shape and size.

The salient object of my invention is to treat piston rings during the manufacture thereof to eliminate strains and irregularities therein to thereby prevent warping and distorting during use and also to very materially reduce the time required in manufacturing articles of this class and in treating or aging them to overcome the warping tendencies.

Another object of my invention is to provide a process of treating piston rings and the like to eliminate warping and distorting tendencies therein, which will be simple and rapid to perform and which can be practiced by manufacturers where time is a material element.

A still further object is to anneal the piston rings or the like to attain uniform hardness throughout and to eliminate hard spots whereby machining will be facilitated.

A selected embodiment of the invention is set forth in the following description wherein reference is made to the accompanying drawing in which

Fig. 1 is an elevational view showing the ring as it appears in the first step of the process;

Fig. 2 illustrates the ring after splitting thereof; and

Fig. 3 is a partially diagrammatic view of the heat treating step in the process of manufacture.

My improved process of manufacture of piston rings embodies four main steps or operations.

The first step in the process consists in casting the piston rings in the usual way and these rings are subsequently machined preferably, though not necessarily, to give a rough finish on the outer peripheries thereof. During such an operation a plurality of rings are usually mounted side by side on a mandrel to expedite the machining. A ring of this character is illustrated in Fig. 1 and is indicated by 4.

The second step in the process consists in transversely slitting the rings to form rings of the so-called split type. The rings 4 are slit diagonally, as indicated at 5, in this step of the process. The process as thus far described does not materially differ from the operations heretofore performed in the manufacture of piston rings.

After the machining and splitting operations have been performed the rings are ready for the third step in the process and in this step the rings are mounted on a non-reciprocating mandrel 6 or the like suspended in a heat-treating chamber 7 which in the present instance is heated by a burner 8 that extends through an opening in the casing 9 which surrounds the chamber 7. The rings 4 on the mandrel 6 are subjected to a temperature of approximately 1100° Fahrenheit, which is above the temperature to which they are subjected during use, for a period of about thirty minutes. The rings are then permitted to cool before the final machine operations are performed. The time of the exposure of the rings to the heat may be lengthened without detrimental effect thereon.

The fourth or final step in the operation is to machine the rings to size, and in this operation any irregularities due to warping or other distorting as a result of the heating and cooling steps are removed.

I have found that articles produced by the

above described process may be machined repeatedly without causing any perceptible warping or distorting, and thus my invention resides primarily in the heat treatment although the heat treatment is but a step in the process of manufacture. With my improved process it is possible to produce accurate and satisfactory rings in three days whereas it would require at least sixty days by the old method and the resulting product would not be as accurate as that produced by my method. Furthermore, since the rings are heated but once appreciable time is saved in the manufacture. Moreover, the fourth or final step in the process may be performed as soon as the rings are cooled after completion of the third step. By heating the rings to a temperature above that to which they are subjected in use, I eliminate the likelihood of the rings being affected by engine heat, that is to say, I prevent additional heat treatment of the rings during use thereof.

While I have particularly described my process in connection with the manufacture of piston rings it is to be understood that this is susceptible to other uses and to variation and modification and I therefore do not wish to be limited to the precise details set forth but desire to avail myself of such changes and alterations as fall within the purview of the following claims.

I claim:

1. The process of treating cast iron piston rings and the like to prevent warping and distorting in use, consisting in arranging the articles on a support and subjecting the same to a temperature of approximately 1100° Fahrenheit for a period of about thirty minutes, and in then allowing the rings to cool to permit finishing of said rings to size as soon as they are cooled.
2. The process of manufacturing piston rings consisting in introducing the rings into a chamber and subjecting the rings but a single time to a temperature above that to which they will be subjected during use, and in then allowing the rings to cool so that further operations may be performed thereon as soon as they are cooled.
3. The process of treating cast iron piston rings and the like consisting in subjecting the rings to a temperature of approximately 1100° Fahrenheit to remove hard spots and other irregularities and prevent warping and distortion in use, and in then allowing the rings to cool to permit finishing of said rings to size as soon as they are cooled.

MARTIN B. COVERT.